



US005431994A

**United States Patent** [19]

Kozulla

[11] **Patent Number:** **5,431,994**[45] **Date of Patent:** **Jul. 11, 1995**[54] **HIGH THERMAL STRENGTH BONDING FIBER**[75] Inventor: **Randall E. Kozulla**, Conyers, Ga.[73] Assignee: **Hercules Incorporated**, Wilmington, Del.[21] Appl. No.: **939,857**[22] Filed: **Sep. 2, 1992****Related U.S. Application Data**

[60] Continuation of Ser. No. 836,438, Feb. 18, 1992, abandoned, which is a division of Ser. No. 474,897, Feb. 5, 1990, abandoned.

[51] **Int. Cl.<sup>6</sup>** ..... **B32B 5/26; D01F 8/06; D04H 1/54; D04H 3/14**[52] **U.S. Cl.** ..... **428/286; 156/62.4; 264/210.6; 264/211; 264/211.14; 264/211.17; 264/234; 428/288; 428/296; 428/373; 428/374**[58] **Field of Search** ..... **428/198, 286, 288, 296, 428/373, 374; 264/211.14, 211.17, 234, 210.6, 211**[56] **References Cited****U.S. PATENT DOCUMENTS**

- 2,335,922 12/1943 Dreyfus .  
 2,715,075 8/1955 Wolinski .  
 2,715,076 8/1955 Wolinski .  
 2,715,077 8/1955 Wolinski .  
 2,985,995 5/1961 Bunting, Jr. et al. .  
 3,364,537 1/1968 Bunting, Jr. et al. .  
 3,428,506 2/1969 Johnstone .  
 3,484,916 12/1969 Johnstone .  
 3,505,164 4/1970 Oppenlander .  
 3,509,013 4/1970 Oppenlander .  
 3,516,899 6/1970 Saunders .  
 3,533,904 10/1970 Jurkiewitsch .  
 3,597,268 8/1971 Smith .  
 3,616,168 8/1971 Johnstone .  
 3,663,675 5/1972 Fukuma et al. .  
 3,693,341 9/1972 Higgins, Jr. .  
 3,807,917 4/1974 Shimoda et al. .  
 3,862,265 1/1975 Steinkamp et al. .  
 3,898,209 8/1975 Watson et al. .  
 3,900,678 8/1975 Aishima ..... 428/374  
 3,907,057 9/1975 Reddekopp .  
 3,907,957 9/1975 Shaffer .

- 4,115,620 9/1978 Gupta et al. .  
 4,134,882 1/1979 Frankfort et al. .  
 4,193,961 3/1980 Roberts .  
 4,195,051 3/1980 Frankfort et al. .  
 4,251,200 2/1981 Parkin .  
 4,259,399 3/1981 Hill .  
 4,303,606 12/1981 Roberts .  
 4,347,206 8/1982 Roberts .  
 4,438,238 3/1984 Fukushima et al. .  
 4,477,516 10/1984 Sugisha ..... 428/373  
 4,480,000 10/1984 Watanabe et al. .  
 4,500,384 2/1985 Tomioka et al. .  
 4,511,615 4/1985 Ohta .  
 4,521,483 6/1985 Sasaki et al. ..... 428/373  
 4,578,414 3/1986 Sawyer et al. .  
 4,592,943 6/1986 Cancian et al. .

(List continued on next page.)

**FOREIGN PATENT DOCUMENTS**

- 2035575 8/1991 Canada .  
 0279511 8/1988 European Pat. Off. .  
 0445536 9/1991 European Pat. Off. .  
 1142065 9/1957 France .  
 18519 3/1973 Japan .  
 092416 4/1991 Japan .  
 34908 1/1957 Luxembourg .  
 738474 10/1955 United Kingdom .  
 2121423 12/1983 United Kingdom .

**OTHER PUBLICATIONS**

Jeffries, R., "Bicomponent Fibres", Merrow Monograph Publ. Co. Ltd., 1971, pp. v & 1-70.  
 English Language abstract of Japanese Patent 48-018519 to Sekisui Chem. Co., Ltd.

(List continued on next page.)

*Primary Examiner*—James C. Cannon  
*Attorney, Agent, or Firm*—Mark D. Kuller; John E. Crowe

[57] **ABSTRACT**

High strength spun melt fiber, preparation thereof utilizing threadline oxidative chain scission degradation of hot fiber spun from polymer component(s) having a broad molecular weight distribution in conjunction with a delayed quench step, and corresponding nonwoven material obtained therefrom.

**110 Claims, 1 Drawing Sheet**

## U.S. PATENT DOCUMENTS

|           |         |                           |
|-----------|---------|---------------------------|
| 4,626,467 | 12/1986 | Hostetter .               |
| 4,632,861 | 12/1986 | Vassilatos .              |
| 4,634,739 | 1/1987  | Vassilatos .              |
| 4,680,156 | 7/1987  | Collier .                 |
| 4,717,325 | 1/1988  | Fujimura et al. .         |
| 4,770,925 | 9/1988  | Uchikawa et al. .         |
| 4,804,577 | 2/1989  | Hazelton et al. .         |
| 4,828,911 | 5/1989  | Morman .                  |
| 4,830,904 | 5/1989  | Gessner et al. .          |
| 4,840,846 | 6/1989  | Ejima et al. .... 428/373 |
| 4,840,847 | 6/1989  | Ohmae et al. .            |
| 4,842,922 | 6/1989  | Krupp et al. .            |
| 4,874,666 | 10/1989 | Kubo et al. .             |
| 4,883,707 | 11/1989 | Newkirk .                 |
| 4,909,976 | 3/1990  | Cuculo et al. .           |
| 5,009,951 | 4/1991  | Ohmae et al. .            |
| 5,066,723 | 11/1991 | Randall, Jr. et al. .     |

## OTHER PUBLICATIONS

- English Language abstract of Japanese Patent 63-061038 to Mitsubishi Petrochemical K.K.
- English Language abstract of Japanese Patent 63-168445 to Chisso Corp.
- English Language abstract of Japanese patent 3-092416 to Daiwa Spinning K.K.
- Deopura et al., "A Study of Blends of Different Molecular Weights of Polypropylene" *Journal of Applied Polymer Science*, vol. 31, 2145-2155 (1986).
- Legare, 1986 TAPPI Synthetic Fibers for Wet System and Thermal Bonding Applications, Boston Park Plaza Hotel & Towers, Boston, Mass., Oct. 9-10, 1986, "Thermal Bonding of Polypropylene Fibers in Nonwovens", pp. 1-13 and attached Tables and Figures.
- Kloos, The Plastics and Rubber Institute, The Conference Department, Fouth International Conference On Polypropylene Fibers And Textiles, East Midlands Conference Centre, Nottinghas, London, UK: Wednesday 23 to Friday 25 Sep. 1987, "Dependence of Structure and Properties of Melt Spun Polypropylene Fibers on Molecular Weight Distribution", pp. i and 6/1-6/10.

Durcova et al., "Structure of Photoxidized Polypropylene Fibers", *Polymer Science U.S.S.R.*, vol. 29, No. 10 (1987), pp. 2351-2357.

Fan et al., "Effects of Molecular Weight Distribution on the Melt Spinning of Polypropylene Fibers", *Journal of Polymer Engineering*, vol. 5, No. 2 (1985) pp. 95-123.

Jeffries, R. "Bicomponent Fibers", Morrow Monograph Publ. Co., 71.

Jones, The Plastics and Rubber Institute, The Conference Department, Fourth International Conference on Polypropylene Fibers and Textiles, East Midlands Conference Centre, Nottinghas, London, UK: Wednesday 23 to Friday 25 Sep. 1987, "A Study of Resin Melt Flow Rate and Polydispersity Effects on the Mechanical Properties of Melt Blown Polypropylene Webs", pp. i and 46/1-46/10.

Mahajan et al., "Fibers Spun From Blends of Different Molecular Weights of Polypropylene", *Journal of Applied Polymer Science*, vol. 43, 49-56 (1991).

Seiler and Goller, "Propylene (PP)" *Kunststoffe* 80 (1990) 10, pp. 1085-1092.

Trent et al., "Ruthenium Tetroxide Staining of Polymers for Electron Microscopy" *Macromolecules*, vol. 16 No. 4, 1983.

Zeicher and Patel, *Proceedings of Second World Congress of Chemical Engineering, Montreal*, vol. 6 (1981) pp. 333-337.



Fig - 1



Fig - 2

## HIGH THERMAL STRENGTH BONDING FIBER

This application is a continuation of application Ser. No. 07/836,438, filed Feb. 18, 1992, which is a division of Ser. No. 07/474,897, filed Feb. 5, 1990, both abandoned.

## BACKGROUND

A number of modern uses have been found for non-woven materials produced from melt spun polymers, particularly degraded polyolefin-containing compositions. Such uses, in general, demand special properties of the nonwoven and corresponding fiber such as special fluid handling, high vapor permeability, softness, integrity and durability, as well as efficient cost-effective processing techniques.

Unfortunately, however, the achievement of properties such as softness, and vapor-permeability, for example, present serious largely unanswered technical problems with respect to strength, durability and efficiency of production of the respective staple and nonwoven products.

One particularly troublesome and long standing problem in this general area stems from the fact that efficient, high speed spinning and processing of polyolefin fiber such as polypropylene requires careful control over the degree of chemical degradation and melt flow rate (MFR) of the spun melt, and a highly efficient quenching step capable of avoiding substantial over- or under-quench leading to melt fracture or ductile failure under high speed commercial manufacturing conditions. The resulting fiber can vary substantially in bonding properties.

It is an object of the present invention to improve control over polymer degradation, spin and quench steps so as to obtain fiber capable of producing nonwoven fabric having increased strength, toughness, and integrity.

It is a further object to improve the heat bonding properties of fiber spun from polyolefin-containing melt such as polypropylene polymer or copolymer.

## THE INVENTION

The above objects are realized by use of the instant process whereby monocomponent or bicomponent fiber having improved heat bonding properties and material strength, elongation, and toughness is obtained by

A. admixing an effective amount of at least one antioxidant/stabilizer composition into a dry melt spun mixture comprising broad molecular weight distribution polyolefin polymer or copolymer, such as polypropylene as hereafter defined, in the presence of an active amount of a degrading composition; various other additives known to the spinning art can also be incorporated, as desired, such as pigments and art-known whiteners and colorants such as TiO<sub>2</sub> and pH-stabilizing agents such as calcium stearate in usual amounts (i.e. 1%-10% or less).

B. heating and spinning the resulting spun melt mixture, at a temperature, preferably within a range of about 250° C.-325° C., and in an environment under sufficient pressure to minimize or control oxidative chain scission degradation of polymeric component(s) within said spun mixture prior to and during said spinning step;

5 C. taking up the resulting hot (essentially unquenched) spun fiber under an oxygen-containing atmosphere maximizing gas diffusion into the hot fiber to effect threadline oxidative chain scission degradation of the fiber; and

10 D. quenching and finishing the resulting partially degraded spun fiber to obtain a raw spun fiber having a highly degraded surface zone of low molecular weight, low birefringence, and a minimally degraded, essentially crystalline birefringent inner configuration, these two zones representing extremes defining an intermediate zone (see below) having a gradation in oxidative degradation depending generally upon fiber structure and rate of diffusion of oxidant into the hot fiber.

15 The resulting fiber or filament is further characterized as the spun product of a broad molecular weight polyolefin polymer or copolymer, preferably a polypropylene-containing spun melt having incorporated therein an effective amount of at least one antioxidant/-stabilizer composition, the resulting fiber or filament, when quenched, comprising, in combination,

20 (a) an inner zone identified by minimal oxidative polymeric degradation, high birefringence, and a weight average molecular weight within a range of about 100,000-450,000 and preferably about 100,000-250,000;

25 (b) an intermediate zone generally externally concentric to the inner zone and further identified by progressive (inside-to-outside) oxidative chain scission degradation, the polymeric material within the intermediate zone having a molecular weight gradation within a range of about 100,000-450,000-to-less than 20,000 and preferably about 10,000-20,000; and

30 (c) a surface zone generally externally concentric to the intermediate zone and defining the external surface of the fiber or filament, the surface zone being further identified by low birefringence, a high concentration of oxidative chain scission degraded polymeric material, and a weight average molecular weight of less than about 10,000 and preferably about 5,000-10,000.

35 Further, the characteristics of the inner zone, the surface zone and the graduated intermediate zone can be defined using terminology which is related to the weight average molecular weight. For example, the various zones can be defined using the melt flow rate of the polymer. In this regard, as the molecular weight decreases towards the surface of the fiber, there will be a corresponding increase in the melt flow rate.

40 For present purposes the term "effective amount", as applied to the concentration of antioxidant/stabilizer compositions within the dry spun melt mixture, is defined as an amount, based on dry weight, which is capable of preventing or at least substantially limiting chain scission degradation of the hot polymeric component(s) within fiber spinning temperature ranges in the substantial absence of oxygen, an oxygen evolving, or an oxygen-containing gas. In particular, it refers to a concentration of one or more antioxidant compositions sufficient to effectively limit chain scission degradation of polyolefin component of a heated spun melt composition within a temperature range of about 250° C. to about 325° C., in the substantial absence of an oxidizing environment such as oxygen, air or other oxygen/nitrogen mixtures. The above definition, however, permits a substantial amount of oxygen diffusion and oxidative

polymeric degradation to occur, commencing at or about the melt zone of the spun fiber threadline and extending downstream, as far as desired, to a point where natural heat loss and/or an applied quenching environment lowers the fiber surface temperature (to about 250° C. or below, in the case of polypropylene polymer or copolymer) to a point where further oxygen diffusion into the spun fiber or filament is negligible.

Generally speaking, the total combined antioxidant-/stabilizer concentration usually falls within a range of about 0.002%-1% by weight, and preferably within a range of about 0.005%-0.5%, the exact amount depending on the particular rheological and molecular properties of the chosen broad molecular weight polymeric component(s) and the temperature of the spun melt; additional parameters are represented by temperature and pressure within the spinnerette itself, and the amount of prior exposure to residual amounts of oxidant such as air while in a heated state upstream of the spinnerette. Below or downstream of the spinnerette an oxygen/nitrogen gas flow ratio of about 100-10/0-90 by volume at an ambient temperature up to about 200° C. plus a delayed quench step are preferred to assure adequate chain scission degradation of the polymer component and to provide improved thermal bonding characteristics, leading to increased strength, elongation and toughness of nonwovens formed from the corresponding continuous fiber or staple.

The term "active amount of a degrading composition" is here defined as extending from 0% up to a concentration, by weight, sufficient to supplement the application of heat to a spun melt mix and the choice of polymer component and arrive at a spinnable (resin) MFR value (preferably within a range of about 5 to 35). Assuming the use of broad molecular weight polypropylene-containing spun melt, an "active amount" constitutes an amount which, at a melt temperature range of about 275° C.-320° C. and in the substantial absence of oxygen or oxygen-containing or -evolving gas, is capable of producing or obtaining a spun melt within the above-stated desirable MFR range.

The term "antioxidant/stabilizer composition", as here defined, comprises one or more art-recognized antioxidant compositions employed in effective amounts as below-defined, inclusive of phenylphosphites such as Irgafos® 168(\*), Ultranox® 626 (commercially available from General Electric), Sandostab PEP-Q(\*\*); N,N'-bis-piperidinyl diamine-containing compositions, such as Chimmassorb® 119 or 944(\*); hindered phenolics, such as Cyanox® 1790(\*\*), Irganox® 1076(\*) or 1425(\*) and the like.

(\*) commercially obtainable as products of Ciba Geigy Corp.

(\*\*) commercially obtainable as products of American Cyanamid Co.

(\*\*3) Commercially obtainable as a product of Sandos Chemical Co.

The term "broad molecular weight distribution", is here defined as dry polymer pellet, flake or grain preferably having an MWD value (i.e. Wt.Avg.Mol.Wt./No.Avg.Mol.Wt.) of not less than about 5.5.

The term "quenching and finishing", as here used, is defined as a process step generic to one or more of the steps of gas quench, fiber draw (primary and secondary if desired) and texturing, (optionally inclusive of one or more of the routine steps of bulking, crimping, cutting and carding), as desired.

The spun fiber obtained in accordance with the present invention can be continuous and/or staple fiber of a (1) monocomponent- or (2) bicomponent-type, the inner zone, in the former, having a relatively high crystallin-

ity and birefringence with a negligible or very modest oxidative chain scission degradation.

In the latter (2) bicomponent type, the corresponding inner layer of the sheath element is comparable to the center cross sectional area of a monocomponent fiber, however, the bicomponent core element of a bicomponent fiber is not necessarily treated in accordance with the instant process or even consist of the same polymeric material as the sheath component, although generally compatible with or wettable by the inner zone of the sheath component.

The sheath and core elements of bicomponent fiber within the present invention can be conventionally spun in accordance with equipment known to the bicomponent fiber art<sup>(\*)4</sup> except for the preferred use of nitrogen or other inert gas environment to avoid or minimize oxygen diffusion into the hot spun melt or the hot core element prior to application of a sheath element around it. In the latter (2) situations (see FIG. 2), the sheath element should possess (a') an inner, essentially crystalline birefringent, non degraded zone contacting the bicomponent core (d'), (b') an intermediate zone of indeterminate thickness and intermediate crystallinity and birefringence, and (c') a highly degraded bicomponent fiber surface zone, the three zones being comparable to the above-described three zones (A'-C') of a monocomponent fiber (see FIG. 1).

(\*4) See, for instance, U.S. Pat. Nos. 3,807,917, 4,251,200 4,717,325 and "Bicomponent Fibers"—R. Jeffries; Merrow Monograph Publishing Company, Pub. 1971

As above noted, the instant invention does not necessarily require the addition of a conventional polymer degrading agent in the spun melt mix, although such use is not precluded by this invention in cases where a low spinning temperature and/or pressure is preferred, or if, for other reasons, the MFR value of the heated polymer melt is otherwise too high for efficient spinning. In general, however, a suitable MFR (melt flow rate) for initial spinning purposes is best obtained by careful choice of a broad molecular weight polyolefin-containing polymer to provide the needed rheological and morphological properties when operating within a spun melt temperature range of about 275° C.-320° C. for polypropylene.

#### BRIEF AND DETAILED DESCRIPTIONS OF DRAWINGS

Some of the features and advantages of the instant invention are further represented in FIGS. 1 and 2 as schematic cross-sections of filament or fiber treated in accordance with applicant's process.

FIG. 1, as shown and above-noted represents a monocomponent-type filament or fiber and FIG. 2 represents a bicomponent-type filament or fiber (neither shown in scale) in which (3) of FIG. 1 represents an approximate oxygen-diffused surface zone characterized by highly degraded polymer of less than about 10,000 (wt Av MW) and preferably falling within a range of about 5,000-10,000 and at least initially with a high smectic and/or beta crystal configuration; (2) represents an intermediate zone, preferably one having a polymer component varying from about 450,000 to about 10,000-20,000 (inside-to-outside), the thickness and steepness of the decomposition gradient depending substantially upon the extended maintenance of fiber heat, initial polymer MWD, the rate of oxidant gas diffusion, plus the relative amount of oxygen residually present in the dry spun mix which diffuses into the hot spun fiber

upstream, during spinning and prior to the take up and quenching steps; inner zone "(1)" on the other hand, represents an approximate zone of relatively high birefringence and minimal oxidative chain scission due to a low or nonexistent oxygen concentration. As earlier noted, this zone usefully has a molecular weight within a range of about 100,000-450,000.

The above three zones within Diagram I, as previously noted are representative of a monocomponent fiber but such zones are usually not visually apparent in actual test samples, nor do they necessarily represent an even depth of oxygen diffusion throughout the treated fiber.

Diagram II represents a bicomponent-type fiber also within the scope of the present invention, in which (4'), (5) and (6) are defined substantially as counterparts of 1-3 of Diagram I while (7) represents a bicomponent core zone which, if desired, can be formed from a separate spun melt composition obtained and applied using a spin pack in a conventional manner<sup>(\*)4</sup>, provided inner 20 layer (4) consists of a compatible (i.e. core-wettable) material. In addition, zone (7) is preferably formed and initially sheath-coated in a substantially nonoxidative environment in order to minimize the formation of a low-birefringent low molecular weight interface between zones (7) and (4).

As before, the quenching step of the spun bicomponent fiber is preferably delayed at the threadline, conveniently by partially blocking the quench gas, and air, ozone, oxygen, or other conventional oxidizing environment (heated or ambient temperature) is provided downstream of the spinnerette, to assure sufficient oxygen diffusion into the sheath element and oxidative chain scission within at least surface zone (c') and preferably both (c') and (b') zones of the sheath element. 25

Yarns as well as webs for nonwoven material are conveniently formed from fibers or filaments obtained in accordance with the present invention by jet bulking, cutting to staple, crimping and laying down the fiber or filament in conventional ways and as demonstrated, for instance, in U.S. Pat. Nos. 2,985,995, 3,364,537, 3,693,341, 4,500,384, 4,511,615, 4,259,399, 4,480,000, and 4,592,943.

While Diagrams I and II show generally circular fiber cross sections, the present invention is not limited to such configuration, conventional diamond, delta, oval, "Y" shaped, "X" shaped cross sections and the like are equally applicable to the instant invention.

The present invention is further demonstrated, but not limited to the following Examples:

#### EXAMPLE I

Dry melt spun compositions identified hereafter as SC-1 through SC-12 are individually prepared by tumble mixing linear isotactic polypropylene flake identified as "A"- "D" in Table I<sup>(\*)5</sup> and having Mw/Mn values of about 5.4 to 7.8 and a Mw range of 195,000-359,000, which are admixed respectively with about 0.1% by weight of conventional stabilizer<sup>(\*)1</sup>. The mix is then heated and spun as circular cross section fiber at a temperature of about 300° C. under a nitrogen atmosphere, using a standard 782 hole spinnerette at a speed of 750-1200 M/m. The fiber thread lines in the quench box are exposed to a normal ambient air quench (cross blow) with up to about 5.4% of the upstream jets in the quench box blocked off to delay the quenching step. The resulting continuous filaments, having spin denier within a range of 2.0-2.6 dpf, are then drawn (1.0

to 2.5×), crimped (stuffer box steam), cut to 1.5 inches, and carded to obtain conventional fiber webs. Three ply webs of each staple are identically oriented and stacked (machine direction), and bonded, using a diamond design calender at respective temperatures of about 157° C. or 165° C., and 240 PLI (pounds/linear inch) to obtain test nonwovens weighing 17.4-22.8 gm/yd<sup>2</sup>. Test strips of each nonwoven (1"×7") are then identically conventionally tested for CD strength<sup>(\*)6</sup> elongation and toughness<sup>(\*)7</sup>. The fiber parameters and fabric strength are reported in Tables II-IV below using the polymers described in Table I in which the "A" polymers are used as controls.

(\*)5 Obtained commercially from Himont Incorporated.

(\*)6 Using a tensile tester of Instron Incorporated.

(\*)7 Energy required to break fabric conventionally, based on stress-strain curve values.

#### EXAMPLE 2 (Controls)

Example I is repeated, utilizing polymer A and/or other polymers with a low Mw/Mn of 5.35 and/or full (non-delayed) quench. The corresponding webs and test nonwovens are otherwise identically prepared and identically tested as in Example 1. Test results of the controls, identified as C-1 through C-9 are reported in Tables II-IV.

TABLE I

| Spun Mix<br>Polymer<br>Identifi-<br>cation | Mw<br>(g/mol) | Sec <sup>(*)8</sup> |       | Intrinsic visc.<br>IV<br>(decileters/g) | MFR<br>(gm/<br>10 min) |
|--------------------------------------------|---------------|---------------------|-------|-----------------------------------------|------------------------|
|                                            |               | Mn<br>(g/mol)       | Mw/Mn |                                         |                        |
| A                                          | 229,000       | 42,900              | 5.35  | 1.85                                    | 13                     |
| B                                          | 359,000       | 46,500              | 7.75  | 2.6                                     | 5.5                    |
| C                                          | 290,000       | 44,000              | 6.59  | 2.3                                     | 8                      |
| D                                          | 300,000       | 42,000              | 7.14  | 2.3                                     | 8                      |

<sup>(\*)8</sup>Size exclusion chromatography

TABLE II

| Melt<br>Sample | Poly-<br>mer | MWD  | Spin<br>Temp<br>°C. |      | Area<br>% Quench Box*  | Comments |
|----------------|--------------|------|---------------------|------|------------------------|----------|
|                |              |      | Blocked             | Off  |                        |          |
| C-1            | A            | 5.35 | 298                 | 3.74 | Control                |          |
| SC-1           | C            | 6.59 | 305                 | 3.74 | 5.5 MWD                |          |
| SC-2           | D            | 7.14 | 309                 | 3.74 | 5.5 MWD                |          |
| SC-3           | B            | 7.75 | 299                 | 3.74 | 5.5 MWD                |          |
| C-2            | A            | 5.35 | 298                 | 3.74 | Control <<br>5.5 MWD   |          |
| C-3            | A            | 5.35 | 300                 | 3.74 | Control <<br>5.5 MWD   |          |
| C-4            | A            | 5.35 | 298                 | 3.74 | Control <<br>5.5 MWD   |          |
| SC-4           | D            | 7.14 | 309                 | 3.74 | No stabilizer          |          |
| SC-5           | D            | 7.14 | 312                 | 3.74 | —                      |          |
| SC-6           | D            | 7.14 | 314                 | 3.74 | —                      |          |
| SC-7           | D            | 7.14 | 309                 | 3.74 | —                      |          |
| SC-8           | C            | 6.59 | 305                 | 5.38 |                        |          |
| SC-9           | C            | 6.59 | 305                 | 3.74 | Control/Full<br>Quench |          |
| C-5            | C            | 6.59 | 305                 | 0    | Control/Full<br>Quench |          |
| C-6            | A            | 5.35 | 290                 | 5.38 | Control <<br>5.5 MWD   |          |
| C-7            | A            | 5.35 | 290                 | 3.74 | Control <<br>5.5 MWD   |          |
| C-8            | A            | 5.35 | 290                 | 0    | Control <<br>5.5 MWD   |          |
| SC-10          | D            | 7.14 | 312                 | 3.74 |                        |          |
| C-9            | D            | 7.14 | 312                 | 0    | Control/Full<br>Quench |          |
| SC-11          | B            | 7.75 | 278                 | 4.03 | —                      |          |
| SC-12          | B            | 7.75 | 299                 | 3.74 | —                      |          |
| SC-13          | B            | 7.75 | 300                 | 3.74 | —                      |          |

TABLE III

| Melt Sample | FIBER PROPERTIES |     |      | Tenacity (g/den) | Elongation % | Comments         |
|-------------|------------------|-----|------|------------------|--------------|------------------|
|             | MFR (dg/min)     | MWD | dpf  |                  |              |                  |
| C-1         | 25               | 4.2 | 2.50 | 1.90             | 343          | Effect of MWD    |
| SC-1        | 25               | 5.3 | 2.33 | 1.65             | 326          |                  |
| SC-2        | 26               | 5.2 | 2.19 | 1.63             | 341          |                  |
| SC-3        | 15               | 5.3 | 2.14 | 2.22             | 398          |                  |
| C-2         | 17               | 4.6 | 2.28 | 1.77             | 310          | Additives Effect |
| C-3         | 14               | 4.6 | 2.25 | 1.74             | 317          | Low MWD          |
| C-4         | 21               | 4.5 | 2.48 | 1.92             | 380          | High MWD         |
| SC-4        | 35               | 5.4 | 2.28 | 1.59             | 407          |                  |
| SC-5        | 22               | 5.1 | 2.33 | 1.64             | 377          | Additives Effect |
| SC-6        | 14               | 5.6 | 2.10 | 1.89             | 357          |                  |
| SC-7        | 17               | 5.6 | 2.48 | 1.54             | 415          |                  |
| SC-8        | 23+              | 5.3 | 2.64 | 1.50             | 327          | Quench Delay     |
| SC-9        | 25               | 5.3 | 2.33 | 1.65             | 326          |                  |
| C-5         | 23               | 5.3 | 2.26 | 1.93             | 345          |                  |
| C-6         | 19               | 4.5 | 2.28 | 1.81             | 360          | Quench Delay     |
| C-7         | 17               | 4.5 | 2.26 | 1.87             | 367          |                  |
| C-8         | 18               | 4.5 | 2.28 | 1.75             | 345          |                  |
| SC-10       | 22               | 5.1 | 2.33 | 1.64             | 377          | Quench Delay     |
| C-9         | 15               | 5.2 | 2.18 | 1.82             | 430          |                  |
| SC-11       | 11               | 5.4 | 2.40 | 2.00             | 356          | —                |
| SC-12       | 15               | 5.3 | 2.14 | 2.22             | 398          |                  |
| SC-13       | 24               | 5.1 | 2.59 | 1.65             | 418          | —                |

TABLE IV

| Melt Sample | FABRIC CHARACTERISTICS<br>(Variation in Calender Temperatures) |                          |             |             |             |
|-------------|----------------------------------------------------------------|--------------------------|-------------|-------------|-------------|
|             | CALENDER Temp (°C.)                                            | FABRIC Weight (g/sq yd.) | CDS (g/in.) | CDE (% in.) | TEA (g/in.) |
| C-1         | 157                                                            | 22.8                     | 153         | 51          | 42          |
| SC-1        | 157                                                            | 21.7                     | 787         | 158         | 704         |
| SC-2        | 157                                                            | 19.2                     | 513         | 156         | 439         |
| SC-3        | 157                                                            | 18.7                     | 593         | 107         | 334         |
| C-2         | 157                                                            | 18.9                     | 231         | 86          | 106         |
| C-3         | 157                                                            | 21.3                     | 210         | 73          | 83          |
| C-4         | 157                                                            | 20.5                     | 275         | 74          | 110         |
| SC-4        | 157                                                            | 18.3                     | 226         | 83          | 102         |
| SC-5        | 157                                                            | 20.2                     | 568         | 137         | 421         |
| SC-6        | 157                                                            | 19.1                     | 429         | 107         | 245         |
| SC-7        | 157                                                            | 21                       | 642         | 136         | 485         |
| SC-8        | 157                                                            | 19.8                     | 498         | 143         | 392         |
| SC-9        | 157                                                            | 21.7                     | 787         | 158         | 704         |
| C-5         | 157                                                            | 19.4                     | 467         | 136         | 350         |
| C-6         | 157                                                            | 19.1                     | 399         | 106         | 233         |
| C-7         | 157                                                            | 19.8                     | 299         | 92          | 144         |
| C-8         | 157                                                            | 17.4                     | 231         | 83          | 105         |
| SC-10       | 157                                                            | 20.2                     | 568         | 137         | 421         |
| C-9         | 157                                                            | 20.4                     | 448         | 125         | 300         |
| SC-11       | 157                                                            | 19.4                     | 274         | 86          | 122         |
| SC-12       | 157                                                            | 18.7                     | 593         | 107         | 334         |
| SC-13       | 157                                                            | 19.4                     | 688         | 132         | 502         |
| C-1         | 165                                                            | 20.3                     | 476         | 98          | 250         |
| SC-1        | 165                                                            | 22.8                     | 853         | 147         | 710         |
| SC-2        | 165                                                            | 19                       | 500         | 133         | 355         |
| SC-3        | 165                                                            | 19.7                     | 829         | 118         | 528         |
| C-2         | 165                                                            | 18.8                     | 412         | 120         | 262         |
| C-3         | 165                                                            | 20.2                     | 400         | 112         | 235         |
| C-4         | 165                                                            | 20.6                     | 453         | 102         | 250         |
| SC-4        | 165                                                            | 19.3                     | 400         | 110         | 239         |
| SC-5        | 165                                                            | 17.9                     | 614         | 151         | 532         |
| SC-6        | 165                                                            | 19.9                     | 718         | 142         | 552         |
| SC-7        | 165                                                            | 20.5                     | 753         | 157         | 613         |
| SC-8        | 165                                                            | 20.4                     | 568         | 149         | 468         |
| SC-9        | 165                                                            | 22.8                     | 853         | 147         | 710         |
| C-5         | 165                                                            | 17.4                     | 449         | 126         | 303         |
| C-6         | 165                                                            | 18.5                     | 485         | 117         | 307         |
| C-7         | 165                                                            | 19.7                     | 482         | 130         | 332         |
| C-8         | 165                                                            | 19.2                     | 389         | 103         | 214         |
| SC-10       | 165                                                            | 17.9                     | 614         | 151         | 532         |
| C-9         | 165                                                            | 19.4                     | 552         | 154         | 485         |
| SC-11       | 165                                                            | 20.1                     | 544         | 127         | 366         |
| SC-12       | 165                                                            | 19.7                     | 829         | 118         | 528         |

TABLE IV-continued

| Melt Sample | FABRIC CHARACTERISTICS<br>(Variation in Calender Temperatures) |                          |             |             |             |
|-------------|----------------------------------------------------------------|--------------------------|-------------|-------------|-------------|
|             | CALENDER Temp (°C.)                                            | FABRIC Weight (g/sq yd.) | CDS (g/in.) | CDE (% in.) | TEA (g/in.) |
| SC-13       | 165                                                            | 19.2                     | 746         | 138         | 576         |

- 5 I claim:
1. A fiber or filament generated from at least one spun melt mixture comprising a broad molecular weight polyolefin polymer or copolymer and containing an effective amount of at least one antioxidant/stabilizer composition, said fiber comprising, in combination,
    - (a) an inner zone identified by minimal oxidative polymeric degradation, high birefringence, and a weight average molecular weight within a range of about 100,000-450,000;
    - (b) an intermediate zone generally externally concentric to said inner zone and further identified by progressive oxidative chain scission degradation with a molecular weight gradation within a range of about 100,000-450,000-to- about 10,000-20,000; and
    - (c) a surface zone generally externally concentric to said intermediate zone and defining the external surface of said fiber, said surface zone being further identified by low birefringence, a high concentration of oxidative chain scission degraded polymeric material, and a weight average molecular weight of less than about 10,000.
  2. A sheath/core bicomponent fiber of claim 1 wherein said inner zone is internally contiguous with and generally externally concentric to a core element.
  3. A fiber or filament of claim 1 wherein said inner zone is an integral part of a monocomponent fiber, formed essentially from a common melt spun mixture.
  4. A fiber of claim 2 wherein the spun melt mixture making up the sheath element comprises polypropylene polymer or copolymer having a broad molecular weight distribution of not less than about 5.5.
  5. A fiber of claim 3 wherein the spun melt mixture comprises polypropylene polymer or copolymer having a broad molecular weight with a molecular weight distribution of not less than about 5.5.
  6. A fiber of claim 4 wherein polymer component of said inner zone of the sheath element has a molecular weight of about 100,000-250,000, degraded polymer component of said intermediate zone has a molecular weight of about 100,000-250,000-to- less than 20,000 and degraded polymer component of said surface zone has a weight average molecular weight of about 5,000-10,000.
  7. A fiber of claim 5 wherein polymer component of said inner zone formed from a common melt spun mixture has a molecular weight of about 100,000-250,000, degraded polymer component of said intermediate zone has a molecular weight of about 100,000-250,000-to-less than 20,000 and said surface zone has a weight average molecular weight of about 5,000-10,000.
  8. A fiber of claim 1 wherein said spun melt mixture contains up to about 1% by weight of at least one antioxidant stabilizer composition.
  9. A polypropylene containing fiber or filament produced by:
    - extruding polypropylene containing material having a molecular weight distribution of at least about 5.5

to form at least one hot extrudate having a surface; and controlling quenching of the at least one hot extrudate in an oxygen containing atmosphere so as to effect oxidative chain scission degradation of the surface to obtain a polypropylene containing fiber or filament having an oxygen degraded surface zone, a substantially non-degraded inner zone and a gradient therebetween. 5

10. The fiber or filament according to claim 9, 10 wherein the polypropylene containing material has a molecular weight distribution of at least about 6.59. 10

11. The fiber or filament according to claim 10, 15 wherein the polypropylene containing material has a molecular weight distribution of at least about 7.15. 15

12. The fiber or filament according to claim 11, 20 wherein the polypropylene containing material has a molecular weight distribution of at least about 7.75. 20

13. The fiber or filament according to claim 9, 25 wherein the polypropylene containing material subjected to extrusion includes a member selected from the group consisting of antioxidants, stabilizers, and mixtures thereof. 25

14. The fiber or filament according to claim 9, 30 wherein the polypropylene containing material subjected to extrusion includes at least one of phenylphosphite and a N,N' bis-piperidinyl diamine derivative. 30

15. The fiber or filament according to claim 13, 35 wherein the polypropylene containing material is extruded from an extruder and said member selected from the group consisting of antioxidants, stabilizers, and mixtures thereof is present in an effective amount to control chain scission degradation of polymeric components in the extruder. 35

16. The fiber or filament according to claim 9, 40 wherein the controlling quenching of the at least one hot extrudate in an oxygen containing atmosphere to effect oxidative chain scission degradation of the surface of the at least one fiber or filament includes controlling the rate of quenching of the hot extrudate. 40

17. The fiber or filament according to claim 16, 45 wherein the controlling quenching comprises delaying quenching of the at least one hot extrudate. 45

18. The fiber or filament according to claim 9, 50 wherein the at least one polypropylene containing fiber or filament comprises a monocomponent or a bicomponent fiber or filament. 50

19. The fiber or filament according to claim 9, 55 wherein the controlling quenching of the at least one hot extrudate in an oxygen containing atmosphere so as to effect oxidative chain scission degradation of the surface comprises maintaining the temperature of the at least one hot extrudate above about 250° C. for a period of time to obtain oxidative chain scission degradation of the surface. 55

20. The fiber or filament according to claim 19, 60 wherein the controlling quenching includes blocking an upper portion of a cross-blow quench. 60

21. The fiber or filament according to claim 19, 65 wherein the controlling quenching includes immediately blocking an area as the at least one extrudate exits a spinnerette. 65

22. The fiber or filament according to claim 19, 70 wherein the controlling quenching includes passing the at least one hot extrudate through a blocked zone. 70

23. The fiber or filament according to claim 22, 75 wherein the blocked zone is open to the oxygen containing atmosphere. 75

24. A polypropylene containing fiber or filament produced by:

extruding polypropylene containing material having a molecular weight distribution of at least about 5.5 to form at least one hot extrudate having a surface, said polypropylene containing material including a member selected from the group consisting of antioxidants, stabilizers, and mixtures thereof; and controlling quenching of the at least one hot extrudate in an oxygen containing atmosphere so as to effect oxidative chain scission degradation of the surface, wherein the controlling quenching comprises maintaining the temperature of the at least one hot extrudate above about 250° C. for a period of time to obtain oxidative chain scission degradation of the surface to obtain a polypropylene containing fiber or filament having an oxygen degraded surface zone, a substantially non-degraded inner zone and a gradient therebetween. 25

25. A polypropylene containing fiber or filament produced by:

extruding a polypropylene containing material having a molecular weight distribution of at least about 5.5 to form at least one hot extrudate having a surface, the polypropylene containing material including a member selected from the group consisting of antioxidants, stabilizers, and mixtures thereof, in an effective amount to control chain scission degradation of polymeric components in the extruder; and

controlling quenching of the at least one hot extrudate in an oxygen containing atmosphere so as to effect oxidative chain scission degradation of the surface, the controlling quenching including maintaining the at least one hot extrudate at a temperature for a sufficient period of time to permit oxidative chain scission degradation of the surface of the hot extrudate to obtain a polypropylene containing fiber or filament having an oxygen degraded surface zone, a substantially non-degraded inner zone and a gradient therebetween. 59

26. A polypropylene containing fiber or filament produced by:

extruding polypropylene containing material having a molecular weight distribution of at least about 5.5 to form at least one hot extrudate having a surface; and

controlling quenching of the at least one hot extrudate in an oxygen containing atmosphere so as to obtain at least one fiber or filament having a surface zone of lower molecular weight and higher melt flow rate than an inner zone of higher molecular weight and lower melt flow rate, and a gradient therebetween comprising a decreasing weight average molecular weight and an increasing melt flow rate towards the surface zone. 78

27. The fiber or filament according to claim 26, 80 wherein the inner zone has a weight average molecular weight of about 100,000 to 450,000 grams/mole. 80

28. The fiber or filament according to claim 27, 85 wherein the inner zone has a weight average molecular weight of about 100,000 to 250,000 grams/mole. 85

29. The fiber or filament according to claim 27, 90 wherein the inner zone has a melt flow rate of 5-25 dg/min. 90

30. The fiber or filament according to claim 27, 95 wherein said surface zone includes the surface of the at least one fiber or filament, and the surface zone has a

weight average molecular weight of less than about 10,000 grams/mole.

31. The fiber or filament according to claim 30, wherein the surface zone has a weight average molecular weight of about 5,000 to 10,000 grams/mole.

32. The fiber or filament according to claim 30, the gradient between said surface zone and said inner zone comprises an intermediate zone positioned between the inner zone and the surface zone having a weight average molecular weight and melt flow rate intermediate 10 the inner zone and the outer zone.

33. The fiber or filament according to claim 30, wherein the inner zone has a high birefringence, and the surface zone has a low birefringence.

34. The fiber or filament according to claim 26, 15 wherein the inner zone has a melt flow rate of 5-25 dg/min.

35. The fiber or filament according to claim 26, wherein the surface zone includes the surface of the at least one fiber or filament, and the surface zone has a 20 weight average molecular weight of less than about 10,000 grams/mole.

36. The fiber or filament according to claim 26, wherein the polypropylene containing material is extruded from an extruder and includes a member selected 25 from the group consisting of antioxidants, stabilizers, and mixtures thereof, in an effective amount to control chain scission degradation of polymeric components of the hot extrudate in the extruder.

37. The fiber or filament according to claim 26, 30 wherein the at least one fiber or filament comprises a monocomponent or a bicomponent fiber or filament.

38. The fiber or filament according to claim 26, wherein the polypropylene containing material has a 35 molecular weight distribution of at least about 6.59.

39. The fiber or filament according to claim 38, wherein the polypropylene containing material has a molecular weight distribution of at least about 7.14.

40. The fiber or filament according to claim 39, wherein the polypropylene containing material has a 40 molecular weight distribution of at least about 7.75.

41. A polypropylene containing fiber or filament produced by:

extruding polypropylene containing material having a molecular weight distribution of at least about 5.5 45 to form at least one hot extrudate having a surface, the polypropylene containing material including a member selected from the group consisting of antioxidants, stabilizers, and mixtures thereof, in an effective amount to control chain scission degradation of polymeric components of the hot extrudate in the extruder; and

controlling quenching of the at least one hot extrudate in an oxygen containing atmosphere so as to obtain at least one fiber or filament having a decreasing weight average molecular weight and an increasing melt flow rate towards the surface of the at least one fiber or filament, the at least one fiber or filament comprising an inner zone having a weight average molecular weight of about 100,000 50 to 450,000 grams/mole; an outer zone, including the surface of the at least one fiber or filament, having a weight average molecular weight of less than about 10,000 grams/mole, and a gradient of weight average molecular weight therebetween. 65

42. The fiber or filament according to claim 41, including the gradient of weight average molecular weight comprises an intermediate zone positioned be-

tween the inner zone and the outer zone having a weight average molecular weight and melt flow rate intermediate the inner zone and the outer zone.

43. The fiber or filament according to claim 41, wherein the polypropylene containing material has a molecular weight distribution of at least about 6.59.

44. The fiber or filament according to claim 43, wherein the polypropylene containing material has a molecular weight distribution of at least about 7.14.

45. The fiber or filament according to claim 44, wherein the polypropylene containing material has a molecular weight distribution of at least about 7.75.

46. A polyolefin polymer fiber or filament produced by:

extruding a mixture comprising a broad molecular weight distribution polyolefin polymer and an effective amount of a member selected from the group consisting of antioxidants, stabilizers, and mixtures thereof under conditions to control oxidative chain scission degradation of polymeric components within the mixture prior to entering an oxygen containing atmosphere as a hot extrudate; and

exposing the hot extrudate to an oxygen containing atmosphere under conditions to effect oxidative chain scission degradation of a surface of the hot extrudate to obtain a highly degraded surface zone of low molecular weight compared to an inner zone of the hot extrudate, and a molecular weight gradient therebetween.

47. The fiber or filament according to claim 46, comprising controlling quenching of the resulting partially degraded extrudate to obtain a fiber or filament having a degraded surface zone of lower molecular weight, and the inner zone having higher molecular weight.

48. The fiber or filament according to claim 47, wherein the mixture contains polypropylene, and has a molecular weight distribution of at least about 5.5.

49. The fiber or filament according to claim 48, wherein the mixture has a molecular weight distribution of at least about 6.59.

50. The fiber or filament according to claim 49, wherein the mixture has a molecular weight distribution of at least about 7.14.

51. The fiber or filament according to claim 50, wherein the mixture has a molecular weight distribution of at least about 7.75.

52. The fiber or filament according to claim 46, wherein the exposing of the hot extrudate to an oxygen containing atmosphere so as to effect oxidative chain scission degradation of the surface comprises maintaining the temperature of the at least one hot extrudate above about 250° C. for a period of time to obtain oxidative chain scission degradation of the surface.

53. The fiber or filament according to claim 52, wherein the controlling quenching includes blocking an upper portion of a cross-blow quench.

54. The fiber or filament according to claim 52, wherein the controlling quenching includes passing the at least one hot extrudate through a blocked zone.

55. The fiber or filament according to claim 54, wherein the blocked zone is open to the oxygen containing atmosphere.

56. A fiber or filament produced by:

extruding a broad molecular weight distribution polyolefin containing material at a temperature and an environment under conditions to control oxida-

tive chain scission degradation of polymeric components within the extruder; exposing resulting hot extrudate to an oxygen containing atmosphere to permit oxygen diffusion into the hot extrudate to obtain oxidative chain scission degradation of a surface of the resulting hot extrudate; and quenching the partially degraded at least one fiber or filament to obtain at least one fiber or filament having a surface zone of lower molecular weight, an inner zone having higher molecular weight than the surface zone, and a molecular weight gradient therebetween.

57. The fiber or filament according to claim 56, wherein the resulting hot extrudate is immediately exposed to an oxygen containing atmosphere.

58. The fiber or filament according to claim 56, wherein the inner zone is substantially not degraded by oxygen.

59. The fiber or filament according to claim 56, wherein the polyolefin containing material contains polypropylene, and has a molecular weight distribution of at least about 5.5.

60. The fiber or filament according to claim 59, wherein the polyolefin containing material has a molecular weight distribution of about 6.59.

61. The fiber or filament according to claim 60, wherein the polyolefin containing material has a molecular weight distribution of at least about 7.14.

62. The fiber or filament according to claim 61, wherein the polyolefin containing material has a molecular weight distribution of at least about 7.75.

63. A fiber or filament, comprising:

a polypropylene containing fiber or filament including a member selected from the group consisting of antioxidants, stabilizers and mixtures thereof having a surface zone comprising an external surface of said fiber or filament, and an inner zone; and said surface zone comprising a high concentration of oxidative chain scission degraded polymeric material as compared to said inner zone, with there being a gradient therebetween, and said surface zone having a weight average molecular weight of less than about 10,000 grams/mole.

64. The fiber or filament according to claim 63, wherein said inner zone is surrounded by said surface zone, said inner zone comprising a minimal concentration of oxidative scission degraded polymeric material, and a weight average molecular weight of about 100,000 to 450,000 grams/mole.

65. The fiber or filament according to claim 64, wherein said inner zone has a weight average molecular weight of about 100,000 to 250,000 grams/mole.

66. The fiber or filament according to claim 63, wherein said surface zone has a weight average molecular weight of about 5,000 to 10,000 grams/mole.

67. The fiber or filament according to claim 66, wherein said inner zone has a weight average molecular weight of about 100,000 to 250,000 grams/mole.

68. The fiber or filament according to claim 67, wherein said gradient comprises an intermediate zone positioned between the inner zone and the surface zone having a weight average molecular weight intermediate the inner zone and the surface zone.

69. The fiber or filament according to claim 63, wherein said surface zone has a low birefringence.

70. The fiber or filament according to claim 64, wherein said surface zone has a low birefringence, and said inner zone has a high birefringence.

71. The fiber or filament according to claim 68, wherein said surface zone has a low birefringence, said inner zone has a high birefringence, and said intermediate zone has a birefringence intermediate the inner zone and the surface zone.

72. A fiber or filament, comprising: a polypropylene containing fiber or filament including a member selected from the group consisting of antioxidants, stabilizers and mixtures thereof having a surface zone comprising an external surface of said fiber or filament, and an inner zone and a gradient therebetween; and

said surface zone comprising a high concentration of oxidative chain scission degraded polymeric material as compared to said inner zone, and said gradient comprising a decreasing weight average molecular weight and an increasing melt flow rate towards the external surface.

73. The fiber or filament according to claim 72, wherein said surface zone has a weight average molecular weight of less than about 10,000 grams/mole.

74. The fiber or filament according to claim 73, wherein said inner zone is surrounded by said surface zone, and comprises a minimal concentration of oxidative scission degraded polymeric material, and having a weight average molecular weight of about 100,000 to 450,000 grams/mole.

75. The fiber or filament according to claim 74, wherein said inner zone has a weight average molecular weight of about 100,000 to 250,000 grams/mole.

76. The fiber or filament according to claim 73, wherein said surface zone has a weight average molecular weight of about 5,000 to 10,000 grams/mole.

77. The fiber or filament according to claim 76, wherein said inner zone has a weight average molecular weight of about 100,000 to 250,000 grams/mole.

78. The fiber or filament according to claim 74, wherein said gradient comprises an intermediate zone positioned between the inner zone and the surface zone having a weight average molecular weight intermediate the inner zone and the surface zone.

79. The fiber or filament according to claim 72, wherein said surface zone has a low birefringence.

80. The fiber or filament according to claim 74, wherein said surface zone has a low birefringence, and said inner zone has a high birefringence.

81. The fiber or filament according to claim 78, wherein said surface zone has a low birefringence, said inner zone has a high birefringence, and said intermediate zone has a birefringence intermediate the inner zone and the surface zone.

82. A fiber or filament comprising:

a polypropylene containing fiber or filaments including a member selected from the group consisting of antioxidants, stabilizers and mixtures thereof comprising an inner zone having a weight average molecular weight of about 100,000 to 450,000 grams/mole; an outer zone, including the surface of the at least one fiber or filament, having a weight average molecular weight of less than about 10,000 grams/mole, and a molecular weight gradient therebetween.

83. A fiber or filament according to claim 82, wherein said gradient comprises an intermediate zone positioned between the inner zone and the outer zone having a

weight average molecular weight and melt flow rate intermediate the inner zone and the outer zone.

84. The fiber or filament according to claim 82, wherein said inner zone has a weight average molecular weight of about 100,000 to 250,000 grams/mole.

85. The fiber or filament according to claim 82, wherein said surface zone has a weight average molecular weight of about 5,000 to 10,000 grams/mole.

86. The fiber or filament according to claim 85, wherein said inner zone has a weight average molecular weight of about 100,000 to 250,000 grams/mole. 10

87. The fiber or filament according to claim 82, wherein said surface zone has a low birefringence, said inner zone has a high birefringence, and said intermediate zone has a birefringence intermediate the inner zone 15 and the surface zone.

88. The fiber or filament according to claim 82, wherein the fiber or filament comprises a monocomponent or a bicomponent fiber or filament.

89. The fiber or filament according to claim 82, including a member selected from the group consisting of antioxidants, stabilizers, and mixtures thereof. 20

90. The fiber or filament according to claim 82, including at least one of phenylphosphite and a N,N'-bis-piperidinyl diamine derivative. 25

91. A fiber or filament comprising:

a thermobondable fiber or filament including a member selected from the group consisting of antioxidants, stabilizers and mixtures thereof comprising an oxygen degraded surface zone, a substantially non-degraded inner zone and a gradient therebetween, and having surface characteristics capable of producing non-woven fabric or material having combined high cross-directional strength and high cross-directional elongation. 30

92. A non-woven fabric or material obtained by bonding at least one web comprised of fiber or filament claimed in claim 1.

93. A non-woven fabric or material obtained by bonding at least one web comprised of sheath/core 40 bicomponent fiber claimed in claim 2.

94. A non-woven fabric or material obtained by bonding at least one web comprised of fiber or filament claimed in claim 3.

95. A non-woven fabric or material obtained by bonding at least one web comprised of fiber claimed in 5 claim 4.

96. A non-woven fabric or material obtained by bonding at least one web comprised of fiber or filament claimed in claim 5.

97. A non-woven fabric or material obtained by bonding at least one web comprised of the fiber or filament claimed in claim 6.

98. A non-woven fabric or material obtained by bonding at least one web comprised of the fiber or filament claimed in claim 7.

99. A non-woven fabric or material obtained by bonding at least one web comprised of the fiber or filament claimed in claim 8.

100. A non-woven fabric or material obtained by bonding the fiber or filament claimed in claim 9.

101. A non-woven fabric or material obtained by bonding the fiber or filament claimed in claim 24.

102. A non-woven fabric or material obtained by bonding the fiber or filament claimed in claim 25.

103. A non-woven fabric or material obtained by bonding the fiber or filament claimed in claim 26.

104. A non-woven fabric or material obtained by bonding the fiber or filament claimed in claim 41.

105. A non-woven fabric or material obtained by bonding the fiber or filament claimed in claim 46.

106. A non-woven fabric or material obtained by bonding the fiber or filament claimed in claim 56.

107. A non-woven fabric or material obtained by bonding the fiber or filament claimed in claim 63.

108. A non-woven fabric or material obtained by bonding the fiber or filament claimed in claim 72.

109. A non-woven fabric or material obtained by bonding the fiber or filament claimed in claim 82.

110. A non-woven fabric or material obtained by bonding the fiber or filament claimed in claim 91.

\* \* \* \* \*